

Patented Sept. 12, 1950

2,522,095

A method of treating cotton fibers and fabrics made therefrom, which consists in subjecting the cotton fibers to a treatment consisting of stretching the fibers, and then subjecting the treated fibers to a treatment consisting of immersing the fibers in a solution of a wetting agent.

# UNITED STATES PATENT OFFICE

2,522,095

## COTTON FIBER TREATMENT

Jack Compton, Rome, Ga., assignor to The B. F. Goodrich Company, New York, N. Y., a corporation of New York

No Drawing. Application May 22, 1945.

Serial No. 595,256

3 Claims. (Cl. 19—66)

2

This invention relates to a method of treating cotton fibers whereby the tensile strength, elasticity and fatigue resistance of such fibers are remarkably increased, to the treated fibers thereby obtained, and to the improved yarns, cords and fabrics prepared from such treated fibers.

In the production of cotton yarns, threads, cords and fabrics from cotton fibers, it has heretofore universally been the practice to pick the cotton fibers from the cotton plant after it has reached maturity, that is, after the cotton bolls have opened, to separate the cotton fibers from the seed by ginning and then to process the fibers by operations known as picking, carding, drawing, combing, slubbing and roving into a form where they may be spun into yarns and then twisted into threads and cords and/or woven into cotton fabrics.

It has been proposed, however, in the copending application of Elmer J. Cerny, Serial No. 460,985 filed Oct. 6, 1942, now Patent No. 2,387,058, Oct. 16, 1945, to modify this procedure by subjecting the cotton fibers prior to the time they are spun into yarn to a stressing process designed to stretch the individual cotton fibers, whereby the tensile strength and fatigue resistance of the fibers themselves and of the yarns and cords subsequently made therefrom are greatly improved.

I have now discovered that far greater improvements in tensile strength and fatigue resistance of the cotton fibers and of the yarns and cords made therefrom may be secured by stretching cotton fibers obtained from unopened cotton bolls rather than mature open cotton bolls, preferably while the natural constituents of the fiber including natural fiber moisture, are retained therein.

By the term "unopened cotton boll" I mean a cotton boll obtained from a cotton plant in that stage of its development between flowering or blossoming and complete maturity when fibers have formed within the bolls and have attained substantially their maximum length and cell wall thickness but the bolls have not yet opened, this stage occurring in general in the last two-thirds of the period between blossoming and maturity, that is, from about 20 days or so after blossoming until opening of the bolls, which occurs at about 45 to 80 days after blossoming depending upon the variety of cotton. Preferably the cotton fibers made use of in this invention are obtained from unopened bolls of the cotton plant during the last third of the period from blossoming until maturity or just a few days before maturity, for example, at 30 or 40 days after blossoming.

5 with certain varieties of cotton which mature at 45 to 50 days after blossoming such as the variety of *Gossypium hirsutum* L. Strain 4 (known as Coker's Super Seven), or at a comparable time in the development of other varieties of cotton, it being understood that the cotton fibers made use of in this invention may be obtained from any of the varieties of the cotton plant (that is, plants of genus *Gossypium* of the family Malvaceae) including the many varieties of *Gossypium barbadense* such as Sea-island and Egyptian and the many varieties of *Gossypium hirsutum* such as New Orleans and Upland, and the like.

10 In the practice of the invention cotton fibers are obtained from cotton plants by picking the unopened bolls from the plants, crushing the bolls, separating the carpels and boll partitions, from the fiber and seed contained therein and finally separating the seed from the fiber. These

15 operations may be effected in any desired manner by hand or by appropriate mechanical devices, it being understood that the particular method and apparatus used in obtaining the cotton fibers from immature unopened cotton bolls are not, in themselves, a part of this invention.

20 One convenient method of obtaining the fibers from unopened cotton bolls consists of picking the bolls from the plants by hand, passing the bolls through crushers and cleaners for the purpose of breaking up the unopened bolls and removing the carpels and boll partitions from the seed and fibers, and then passing the seed and fibers through a gin to remove the seed from the fibers.

25 After securing the cotton fibers from unopened cotton bolls, these may then be subjected to operations, such as drawing and combing, designed to arrange the fibers in a parallel relation, before proceeding to the next step of stretching the fibers. It is preferred to carry out these operations, as well as the previous operation of removing the seeds from the fiber, as soon as possible after opening of the bolls and in a moist atmosphere in order to prevent the removal of the natural moisture from the cotton fibers. Aqueous solutions of wetting agents may also be added to the cotton before the stretching process, if desired, but it is preferred that the cotton be in a condition such that it has retained its natural moisture

30 and the use of wetting agents is therefore unnecessary.

35 The stretching of the cotton fibers from unopened cotton bolls, preferably while moist with their natural moisture, may be effected by firmly gripping the ends of the individual fibers and

applying to one of the gripped ends a tension less than the breaking strength of the fibers. Preferably the tension applied is from 25 to 75% of the breaking strength of the fibers, and is applied for a short duration only, after which the tension is released and the tensioning repeated, if desired, so long as the total effect is not to break the fibers. One method of applying tension to the individual fibers is to prepare fiber bundles and mount these bundles in steel grips a distance apart such that each fiber is firmly gripped, and then to suspend a weight from the gripped bundles. Another method, better adapted for extensive use, is to pass a sliver of paralleled fibers through successive pairs of rolls of equal weight and spaced apart a distance less than fiber length so that the ends of the individual cotton fibers in the sliver are simultaneously gripped with substantially equal forces by the two pairs of rolls, while rotating the second or delivering pair of rolls at a peripheral speed greater than the first or entering pair of rolls so that tension is applied to the individual fibers as they are gripped by the rolls, and the fibers are stretched upon passage of the sliver through the rolls.

After stretching of the fibers, they may be dried, under tension if desired, and allowed to recover in a standard atmosphere. They are then ready to be subjected to any of the ordinary operations in producing cords, yarns, fabrics and other fibrous structures from cotton fibers. For example they may be spun into yarn and twisted into tire cords which possess tensile strength and fatigue resistance much higher than cords of similar construction prepared from untreated mature cotton fibers obtained from open cotton bolls and even higher than cords of similar construction prepared from mature cotton fibers similarly obtained, which have been stretched in the same way.

As an example of the invention, further illustrating the advantages thereof, a quantity of cotton fibers were obtained from cotton plants of the variety known as Coker's Super Seven at 40 days after blossoming of the cotton, by picking the unopened bolls from the plant and separating the cotton fibers from the carpels and seeds. These 40-day cotton fibers, which possessed an average fiber length of  $1\frac{1}{8}$ ", were then arranged in parallel relation and prepared into fiber bundles weighing 5 mg. and consisting of about 1500 individual fibers. The fiber bundles were then mounted in steel grips, the distance between the grips being  $3/16$ ", so that each individual fiber was firmly gripped. The tensile strength of a number of these bundles was determined by means of a Suter tensile testing machine and was found to average 13.1 lbs. for conditioning cotton. The fatigue resistance of the fiber bundles was also determined by allowing the gripped fiber bundle to be vibrated under a load of 2.5 lbs. at room temperature until breakage of the fibers occurred, and the fatigue life was found to be 8.1 hours for conditioned cotton.

Fiber bundles of the 40-day cotton, while still wet from the bolls, were then stretched by suspending a 5 lb. weight from the gripped fiber bundles under static conditions for 30 seconds,

and then allowing the fibers to dry under a 4 lb. load for 2 hours. The fibers were then conditioned in a standard atmosphere for 24 hours, and the tensile strength and fatigue resistance then determined as before. It was found that the tensile strength of the 40-day cotton had been increased from 13.1 lbs. to 24.0 lbs. by the stretching process and that the fatigue life had been increased from 8.1 hours to 68.5 hours.

In another example of the invention, 30-day cotton fibers from Coker's Super Seven cotton were treated in the same manner and it was found that stretching of the fibers increased the tensile strength from 12.0 to 25.1 lbs. and increased the fatigue life from 23.5 to 42.1 hours.

When fully matured cotton fibers of the same variety were stretched in the same manner, however, the increase in tensile strength was only from 14.2 to 16.9 lbs. and the increase in fatigue life was only from 19.6 hrs. to 26.2 hrs. It is thus seen that stretching of immature fibers is far more effective in improving tensile strength and fatigue resistance than is stretching of mature fibers and that the former yields fibers having much greater tensile strength and fatigue resistance after stretching than does the latter.

Having thus described my invention it is my desire that it be construed broadly, limited only by the spirit and scope of the appended claims.

I claim:

1. The method which comprises obtaining cotton fibers from unopened bolls, subjecting the individual fibers to a tension of 25 to 75% of the breaking strength of said fibers in a moist atmosphere while maintaining the natural moisture content of said fibers, releasing said tension, drying said fibers, and allowing said fibers to recover.

2. The method which comprises obtaining cotton fibers from unopened bolls, wetting said fibers with water, subjecting the wetted individual fibers to a tension of 25 to 75% of the breaking strength of said fibers, releasing the tension, drying said fibers, and allowing said fibers to recover.

3. The method which comprises obtaining cotton fibers from unopened bolls, arranging a multiplicity of said fibers in substantially parallel relation, subjecting the individual fibers while so arranged and while maintaining the natural moisture content of said fibers to a tension of 25 to 75% of the breaking strength of said fibers, releasing said tension, and allowing said fibers to recover.

JACK COMPTON.

#### REFERENCES CITED

The following references are of record in the file of this patent:

#### UNITED STATES PATENTS

| Number    | Name            | Date          |
|-----------|-----------------|---------------|
| 1,689,443 | MacGregor       | Nov. 30, 1928 |
| 1,846,467 | Benjamin        | Feb. 23, 1932 |
| 1,870,039 | Conrad          | Aug. 2, 1932  |
| 2,103,218 | Gwaltney et al. | Dec. 21, 1937 |
| 2,220,958 | Jennings        | Nov. 12, 1940 |
| 2,387,058 | Cerny           | Oct. 16, 1945 |

#### OTHER REFERENCES

"Cotton Manufacturing," Part 2, by E. A. Posselt, published by E. A. Posselt, Philadelphia, Pennsylvania.